

## UNITED STATES PATENT OFFICE

CHARLES H. PRITHAM, OF UPPER DARBY, PENNSYLVANIA

## PRIMER COMPOSITION

No Drawing.

Application filed December 1, 1926. Serial No. 152,053.

(GRANTED UNDER THE ACT OF MARCH 3, 1883, AS AMENDED APRIL 30, 1928; 370 O. G. 757)

The invention described herein may be manufactured and used by or for the Government for governmental purposes without the payment to me of any royalty thereon.

The subject of this invention is a primer composition.

The priming compositions heretofore used in this country have contained potassium chlorate as one of their principal oxidizing ingredients. The employment of this salt is highly undesirable owing to the fact that when the primer is fired potassium chloride is formed which is deposited in the bore of the gun and if not carefully removed will cause corrosion and pitting.

The problem has been successfully met for many years in foreign countries by substituting barium nitrate for the potassium chlorate but the use of such improved composition is only possible in certain types of primers such as the Berdan primer, in which the anvil is contained in the cartridge itself providing considerable space in the primer cup and allowing the use of a sufficient quantity of the primer mixture.

Because the barium mixture is more bulky than the potassium mixture it can not be successfully employed in the type of primer used in small arms cartridges of American manufacture in which the anvil occupies part of the space in the primer cup.

I have discovered that the barium nitrate primer mixture above referred to may be modified to give successful results in less than normal charges by incorporating in the mixture a small percentage of high explosive consisting of nitrated hydrocarbons or aromatics such as trinitrotoluol, trinitrobenzene, trinitroaniline, trinitroanisole, pentaerythritetranitrate or the like.

The amount of high explosive incorporated in the primer varies with the nature of the high explosive used but is generally from 4 to 8%.

A typical example of a non-corrosive

primer composition which has been successfully used is in part the standard Swiss primer mixture and has approximately the following composition:

|                                       | Per cent  |
|---------------------------------------|-----------|
| Fulminate of mercury-----             | 37 50     |
| Barium nitrate-----                   | 32        |
| Antimony sulphide-----                | 28        |
| Ground glass-----                     | 3         |
| To which is added high explosive----- | 4 to 8 55 |

I claim:

A primer mixture consisting of fulminate of mercury 37 parts, barium nitrate 32 parts, antimony sulphide 28 parts, ground glass 3 parts, and a high explosive 4 to 8 parts.

CHARLES H. PRITHAM.

65

70

75

80

85

90